

[54] WATER RESISTING AND  
ANTICORROSION PAINT VEHICLE[75] Inventors: Satoru Enomoto; Hisayuki Wada;  
Mikio Fujioka; Masao Koguro, all of  
Fukushima, Japan[73] Assignee: Kureha Kagaku Kogyo Kabushiki  
Kaisha, Tokyo, Japan

[22] Filed: July 23, 1970

[21] Appl. No.: 57,666

## [30] Foreign Application Priority Data

July 23, 1969 Japan ..... 44/57625

[52] U.S. Cl. .... 208/14, 208/44, 260/667,  
260/671 G, 260/33.6

[51] Int. Cl. .... C10g 39/00

[58] Field of Search..... 208/14, 49, 62, 143, 144, 22,  
208/44; 260/667

## [56] References Cited

## UNITED STATES PATENTS

2,910,426 10/1959 Gluesenkamp et al..... 208/143

Primary Examiner—Herbert Levine

Attorney—Sughrue, Rothwell, Mion, Zinn and Mac-  
peak

## [57] ABSTRACT

A paint vehicle comprising a hydrocarbon compound having a specific gravity of from 0.92 to 1.0, a mean molecular weight of from 200 to 1000 measured by a vapor pressure osmotic pressure method, an aromatic C-H proton density of less than 3 percent, said aromatic C-H proton having a  $\tau$  value of less than 4 determined by nuclear magnetic resonance absorption spectrum, and a transparency such that the percent transmittance of a 10 percent hexane solution thereof, measured by the absorption of visible light of wavelengths longer than 500  $\text{m}\mu$ , is higher than 60 percent.

2 Claims, 3 Drawing Figures



PATENTED JAN 30 1973

3,714,020



FIG. 1



FIG. 2



FIG. 3

INVENTORS

SATORU ENOMOTO, HISAYUKI WADA,  
MIKIO FUJIOKA, MASAO KOGURO

BY Sughrue, Rothwell, Mion, Zinn & Macpeak ATTORNEYS

## WATER RESISTING AND ANTICORROSION PAINT VEHICLE

### BACKGROUND OF THE INVENTION

#### 1. Field of the Invention

The present invention relates to a novel paint vehicle, the vehicle comprising a naphthenic compound which is almost colorless and transparent and one which has water resisting and anticorrosive properties.

#### 2. Description of the Prior Art

In general, resins having so-called three-dimensionally cross-linked structures, such as alkyd resins, epoxy resins, urethane resins, etc., have been known to have excellent properties as coating materials but since they are insufficient in water resisting and anticorrosive properties, it has been strongly desired to improve such properties. On the other hand, from the viewpoint of application of painting materials, the development of a paint vehicle which can be painted as thick as possible by one painting operation has also been strongly desired in this field.

Hitherto, as materials for satisfying both of the above demands, coal tar and coal pitch have been employed as paint vehicles. However, coal tar and coal pitch have such faults that since they are black, the use thereof is limited to a narrowed range and also it is quite difficult to supply these materials having constant qualities successively. Furthermore, since impurities originating from the coal used as the raw material inevitably occur in the vehicle, the stability during preservation is reduced and also they give off specific odors, which in turn results in various disadvantages from the aspects of working properties and sanitation. Moreover, a painting material containing coal tar or coal pitch has the further disadvantage that when the coating material is practically applied and subjected to outdoor exposure for a long period of time, the gloss of the coating is degraded, a chalking phenomenon occurs, and the mechanical properties are greatly reduced.

Therefore, a principal object of the present invention is to provide a paint vehicle which can provide to the paint such advantages as a high water-resisting property, a suitable anticorrosive property and thick paintability.

### SUMMARY OF THE INVENTION

The present invention provides a paint vehicle comprising hydrocarbon compounds having the following characteristics:

- a. a transparency such that the present transmission of a 10 percent hexane solution thereof, measured by the absorption of visible light of a wavelength longer than 500 m $\mu$ , is higher than 60 percent;
- b. a mean molecular weight of from 200 to 1,000, measured by a vapor pressure osmotic pressure method (hereinafter referred to as the VPO method);
- c. a specific gravity of 0.92 to 1.0; and
- d. an aromatic C—H proton density of less than 3 percent, determined by means of a high resolving power, nuclear magnetic resonance absorption spectrum (wherein the  $\tau$  value of tetramethylsilane is defined to be 10 as a standard, a  $\tau$  value less than 4 is the aromatic C—H proton, and a value of 4 to 10 is the alkyl chain proton and the methylene proton), hereinafter referred to as NMR. See

FIGS. 1 and 2 for a graphic analysis of the aromatic C—H proton density requirement.

From the results of measurements by various analytical means and the results of measuring physical properties, the hydrocarbon compounds of the present invention are assumed to be composed of a group of compounds in which an alkyl group having less than eight carbon atoms, and preferably less than four carbon atoms, has been added to a compound having at least two naphthene rings combined in linear fashion, a compound wherein at least two naphthene rings have been condensed, or a compound wherein single ring naphthenic compounds have been linearly combined. However, since an overall conclusive analysis of the hydrocarbon compounds of the present invention cannot be performed, the compositions of the hydrocarbon compounds have not yet been confirmed. Therefore, as a measure of the naphthene rings which are the principal features of the vehicle of this invention, the presence of aromatic rings by measuring the NMR is limited to the procedure as described above (i.e., the percentage of the aromatic C—H proton density).

### BRIEF DESCRIPTION OF THE DRAWINGS

FIG. 1 is a graph showing the NMR spectrum of the vehicle of the present invention;

FIG. 2 is a graph showing the NMR spectrum of a substance having an aromatic C—H proton density higher than 3 percent, which is outside the scope of this invention; and

FIG. 3 is a graph showing the visible spectrum of both the vehicle of this invention and the substance characterized in FIG. 2.

### DETAILED DESCRIPTION OF THE PREFERRED EMBODIMENTS

As is clear from the results shown in FIG. 3, curve 2, the substance shown in FIG. 2, is colored.

Also, the vehicle of this invention is utterly different from alkyl naphthenic compounds such as liquid paraffin; in particular, the former has a larger specific gravity and is more compatible with resins than the latter. This is astonishing when it is considered that liquid paraffins show less of a miscibility with resins as additives for coating compositions.

The degree of transparency of the vehicle of this invention when shown by the Gardner color number is less than 8, and this is so defined in this invention that the percent transmittance of a solution prepared by dissolving 10 g of the vehicle of this invention in 100 ml of hexane or tetrahydrofuran, measured by the absorption of visible light of wavelengths longer than 500 m $\mu$ , is higher than 60 percent, and preferably higher than 80 percent. This is also clearly confirmed by the fact that the vehicle is colored by increasing the proportion of the aromatic C—H protons of the aromatic rings as shown in FIGS. 1-3. Also, it is preferable that the softening point of the vehicle of this invention be in a range of 25°-100° C as a solid and the viscosity thereof as a liquid at 25° C be 1,000-50,000 cps.

The aforesaid vehicle of the present invention is colorless and transparent but may be colored by coloring materials such as pigments, etc.

Furthermore, the vehicle of this invention has no bad odor as does coal tar, etc., and has very few aromatic

rings in its structure, and thus, the vehicle is harmless to both humans and animals and also has no bad influences on the work property of the paint. In addition, it also has a sufficient compatibility with resins, water resisting property, weathering resisting property, anticorrosive property and a thick paintability. Therefore, the vehicle of the present invention overcomes the above-mentioned disadvantages without losing the merits of coal tar or coal pitch.

The vehicle of this invention may be prepared by hydrogenating the aromatic rings of hydrocarbon compounds containing a large amount of aromatic rings (i.e., more than two rings). As such hydrocarbon compounds, there are illustrated coal tars, various residual oils obtained in petroleum refining treatments (e.g., visbraker residual oil, coker residual oil, catalytic cracking cycle oil, dealkylation residual oil, etc.), high temperature cracked residual oils of petroleum (e.g., bottom oil recovered during the production of ethylene by the cracking of naphtha, tars recovered during the production of ethylene-acetylene, and oil tars by-produced by the high temperature gasification cracking of petroleum crude oil, heavy oil, etc.), and the like.

Moreover, for improving the flexibility and compatibility in the painting properties of the vehicle, it is possible as the case may be to conduct the nucleus hydrogenation of the feed stock after alkylating the aforesaid hydrocarbons with olefins having less than eight carbon atoms, preferably less than four carbon atoms. The nucleus hydrogenation may be conducted using a catalyst and apparatus employed for ordinary hydrogenation processes. In this case, however, it is preferable to conduct, before the hydrogenation, a desulfurization step, which is generally used for removing impurities which may poison the catalyst.

The desulfurization may be conducted in a conventional manner using a known desulfurization apparatus. The catalyst to be employed in the desulfurization step involves cobalt, molybdenum or nickel in the form of metals, oxides, sulfides, or combinations thereof which may be supported by suitable carriers such as alumina and silica-alumina. The desulfurizing reaction is carried out at a temperature of 350° to 450° C under a pressure of 20-100 kg/cm<sup>2</sup> using a feed ratio (molar ratio of hydrogen to tar fraction) of 3-20 moles/mole, at a liquid hourly space velocity of 0.5-10 cc/cc-cat/hr (L.H.S.V.). Under such conditions, the reaction takes place readily to attain good desulfurization of the sulfur contained in the tar fractions.

The subsequent alkylation reaction is conducted by mixing the gaseous olefins with the tar fraction and reacting them in the presence of a suitable catalyst. The catalyst to be employed preferably includes a silica-alumina type catalyst or a metal belonging to Group III-B of the Periodic Table, such as lanthanum, cerium, thorium, etc., carried by a suitable carrier such as zeolite.

The feed olefin to be used is preferably a lower olefin generally having not more than eight carbon atoms, preferably two to four carbon atoms. Typical olefins to be used are ethylene, propylene, butylene. The use of such olefins is economically advantageous. The reaction conditions to be employed are as follows: a temperature between 150° C and 380° C, a pressure between 1 and 50 kg/cm<sup>2</sup>, a feed ratio between 0.2 and

10 moles of olefin per mole of the tar fraction and a liquid hourly space velocity of from 0.1 to 50 cc/cc-catalyst/hr.

The reaction takes place readily with the use of the catalyst and is conducted over a prolonged period of time without decrease of the activity of the catalyst.

Since the tar fractions have very few side chains, an alkyl side chain may be added under desired control. The length of the alkyl group to be added depends upon the kind of olefin to be used and the degree of alkylation (the moles of olefin to be reacted per mole of the tar fraction) can be increased by employing a high feed ratio or by employing a small liquid hourly space velocity. The alkylated tar thus formed has a lower specific gravity and refractive index as well as a higher H/C, viscosity, average molecular weight and boiling point than those of the feed tar fraction. Through analysis of the alkylated product by means of gas chromatography, infrared absorption spectrum or nuclear magnetic resonance absorption spectrum, etc., the alkylated tar is estimated to have a chemical structure consisting of condensed polycyclic aromatic rings having from two to five, preferably from two to four, aromatic rings which are combined with added alkyl groups having the same carbon number as that of the olefin used in the reaction.

The subsequent hydrogenation reaction is carried out by admixing the alkylated tar with hydrogen and reacting them in the presence of a suitable catalyst. The catalyst to be used in the hydrogenation process includes the metals belonging to Groups VI, VII, and VIII, and oxides and sulfides thereof, and combinations of them. These components may be supported by carriers such as diatomaceous earth, alumina, bauxite, pumice stone, silica alumina, activated carbon, etc. Typical examples of these catalysts are nickel-carrying diatomaceous earth, molybdenum-carrying alumina, platinum-carrying alumina, cobalt-carrying alumina, etc. The reaction is carried out under the following conditions: a temperature of 100°-450° C, a pressure of 10-300 kg/cm<sup>2</sup>, a feed rate of hydrogen of 5-30 moles per mole of alkylated tar and a liquid hourly space velocity of 0.5-10 cc/cc-catalyst/hr. The reaction in this step involves mainly the hydrogenation of the polycyclic aromatic compounds not accompanied by such side reactions as the dissociation of the alkyl side chain, the ring opening of the naphthene rings, decomposition, polymerization, etc., thus forming alkylated polycyclic naphthene compounds in good yield. By removing fractions having boiling points of lower than 250°-300° C, calculated at normal pressure, from the reaction product thus obtained, the vehicle of this invention can be obtained.

The paint vehicle of this invention gives particularly excellent effects as painting materials to resins having three-dimensionally cross-linked structures by curing. As these resins, there may be illustrated the following: alkyl resins, urethane resins, epoxy resins, epoxy-urethane resins, alkyl-urethane resins, esterified epoxy resins, epoxy-alkyl resins, and the like.

By using 5-500 parts by weight of the vehicle of this invention to 100 parts by weight of the aforesaid resin, effective water resisting and anticorrosive properties can be obtained. Moreover, in the case of employing expensive resins such as epoxy resins and urethane

resins, by using a properly large amount of the vehicle, the cost of the paint may be reduced without degrading the properties of the resin itself. The above-mentioned vehicle, relating to the present invention, may be optionally blended with either prepolymers or hardening agents for the epoxy resin or urethane resin without any trouble.

Furthermore, when a painting material is prepared from the resin and the vehicle of this invention, a solvent may be used for facilitating the painting operation. As such a solvent, there are illustrated aromatic, aliphatic and alicyclic hydrocarbons; ketones such as methyl ethyl ketone, methyl isobutyl ketone, cyclohexanone; esters such as ethyl acetate, amyl acetate, etc.; cyclic ethers such as tetrahydrofuran, dioxane etc.; and chlorine-containing compounds such as carbon tetrachloride, ethylene dichloride, etc. These solvents may be used alone or as mixtures thereof according to the purpose and uses thereof.

The vehicles of this invention may further be modified by adding various conventional additives such as a plasticizer, a softening agent, a filler, a curing agent, a curing accelerator, an antioxidant, a colorant, etc.

The invention will now be explained further by referring to the following examples, which are deemed to be merely illustrative, and not limiting, in nature.

#### EXAMPLE 1

A tarry material prepared by pyrolyzing Seria crude oil at 1,300° C and at a contact time of 0.002 second was subjected, respectively, to desulfurization, alkylation by butylene, and nucleus hydrogenation under the conditions shown below and then, by removing fractions having boiling points lower than 400° C, calculated at normal pressure, vehicle A of this invention was obtained.

| Reaction Catalyst                                      | Desulfurization Co-Ni-alumina<br>3:7:90 (by weight) | alkylation silica-alumina<br>85:15 (by weight) | Nucleus hydrogenation Ni-diatomaceous earth<br>40:60 (by weight) |
|--------------------------------------------------------|-----------------------------------------------------|------------------------------------------------|------------------------------------------------------------------|
| pressure<br>kg/cm <sup>2</sup> -gauge                  | 40                                                  | 30                                             | 180                                                              |
| temperature<br>(°C)                                    | 400                                                 | 200                                            | 300                                                              |
| liquid hourly space<br>velocity<br>(cc/cc-catalyst/hr) | 0.5                                                 | 2.0                                            | 1.0                                                              |
| butylene/raw<br>material<br>(mole ratio)               | —                                                   | 5                                              | —                                                                |
| hydrogen/raw<br>material<br>(mole ratio)               | 5                                                   | —                                              | 10                                                               |
| butylation<br>degree<br>(mol/mol-tar)                  | —                                                   | 2.1                                            | —                                                                |

The general properties of vehicle A thus obtained were as follows:

|                                     |       |
|-------------------------------------|-------|
| Specific gravity                    | 0.990 |
| Softening point                     | 32 °C |
| NMR aromatic C—H proton density (%) | 0     |

|                                                                     |      |
|---------------------------------------------------------------------|------|
| Visible percent transmittance of 10% hexane solution at 500 m $\mu$ | 93 % |
| Mean molecular weight (VPO)                                         | 420  |

5 The NMR spectrum of vehicle A is shown in FIG. 1 of the accompanying drawings. Also, the percent transmittance is shown in FIG. 3 as curve 1.

#### EXAMPLE 2

10 A bottom oil obtained from the high-severity ethylene cracking of petroleum naphtha was subjected to desulfurization, alkylation by ethylene, and nucleus hydrogenation under the conditions shown in the following table. By removing fractions having boiling points of lower than 400° C, calculated at normal pressure, the vehicle B of this invention was obtained.

| Reaction Catalyst                                    | desulfurization<br>Co-Mo-alumina<br>5:5:90<br>(by weight) | alkylation<br>silica-alumina<br>85:15<br>(by weight) | Nucleus hydro-<br>genation<br>Ni-alumina<br>40:60<br>(by weight) |
|------------------------------------------------------|-----------------------------------------------------------|------------------------------------------------------|------------------------------------------------------------------|
| pressure<br>(kg/cm <sup>2</sup> -G)                  |                                                           | 40                                                   | 40                                                               |
| temperature<br>(°C)                                  | 400                                                       | 400                                                  | 250                                                              |
| liquid hourly space<br>velocity (cc/cc-catalyst/hr)  | 0.5                                                       | 0.5                                                  | 1.0                                                              |
| ethylene/raw<br>material<br>(mole ratio)             | —                                                         | 10                                                   | —                                                                |
| hydrogen/raw<br>material<br>(mole ratio)             | 5                                                         | —                                                    | 10                                                               |
| butylation<br>degree<br>(moles/moles<br>-bottom oil) | —                                                         | 1.8                                                  | —                                                                |

The general properties of vehicle B are as follows:

|    |                                                                     |           |
|----|---------------------------------------------------------------------|-----------|
| 40 | Specific gravity                                                    | 0.975     |
|    | Viscosity                                                           | 4,500 cps |
| 50 | NMR aromatic C—H proton density (%)                                 | 0.5       |
|    | Visible percent transmittance of 10% hexane solution at 500 m $\mu$ | 82 %      |
| 45 | Mean molecular weight (V.P.O.)                                      | 380       |

#### EXAMPLE 3

50 A bottom oil obtained from a low-severity ethylene cracking of petroleum naphtha was subjected to desulfurization and nucleus hydrogenation under the conditions shown in the following table. By removing fractions having boiling points of lower than 380°C, calculated at normal pressure, vehicle C of this invention was obtained.

| Reaction Catalyst | Desulfurization Co-Ni-alumina<br>3:7:90 (by weight) | Nucleus hydrogenation<br>Ni-diatomaceous earth<br>40:60 (by weight) |
|-------------------|-----------------------------------------------------|---------------------------------------------------------------------|
| 60                | pressure<br>(kg/cm <sup>2</sup> -G)                 | 50                                                                  |
|                   | temperature<br>(°C)                                 | 400                                                                 |
| 65                | liquid space<br>velocity<br>(cc/cc-catalyst/hr)     | 0.5                                                                 |
|                   | hydrogen/raw<br>material<br>(mole ratio)            | 5                                                                   |

The general properties of vehicle C of this invention prepared above are as follows:

|                                                                     |           |
|---------------------------------------------------------------------|-----------|
| Specific gravity                                                    | 0.965     |
| Viscosity                                                           | 4,000 cps |
| NMR aromatic C-H proton density                                     | 1.0%      |
| Visible percent transmittance of 10% hexane solution at 500 m $\mu$ | 98%       |
| Mean molecular weight (VPO)                                         | 330       |

#### EXAMPLE 4

Each of vehicles A, B and C of this invention prepared in Examples 1, 2 and 3, respectively, was blended in an epoxy resin to provide a painting material and the tests shown in Table 1 were conducted using the painting material thus prepared. The compositions

The above test was made according to JIS-K-5400.

#### EXAMPLE 5

Each of vehicles A, B and C prepared in Examples 1, 2 and 3, respectively, was blended with an alkyd resin (as shown below) and the properties of the painting material thus prepared were investigated. In the test procedures, the painted material having the following composition was employed.

10

#### Composition 3

|                                                         |                      |
|---------------------------------------------------------|----------------------|
| Vehicle of the present invention                        | 100 parts(by weight) |
| Vecosol P470-70 (made by Nippon reichhold)              | 100 parts(by weight) |
| Mixture of cobalt naphthenate and manganese naphthenate | 5 "                  |

15

TABLE 2

| Vehicle | Compo-<br>sition | Test method                       |                                 |                                 |                          |                              |                                                           |             |
|---------|------------------|-----------------------------------|---------------------------------|---------------------------------|--------------------------|------------------------------|-----------------------------------------------------------|-------------|
|         |                  | **a                               | b                               | c                               | d                        | e                            | f                                                         | g           |
|         |                  | One year<br>in distilled<br>water | Fade-O-meter,<br>2,000 hrs.     | Outdoor exposure<br>for 1 year  | 3/16" mandrel<br>100/100 | Du Pont type, 0.5 kg.-50 cm. |                                                           | Pen-<br>cil |
| A.....  | 3                | Unvaried                          | Not inferior to control sample. | Not inferior to control sample. | Endured                  | Passed                       | Neither cracked nor stripped by the impact of the weight. | H           |
| B.....  | 3                | do                                | do                              | do                              | do                       | do                           | do                                                        | H           |
| C.....  | 3                | do                                | do                              | do                              | do                       | do                           | do                                                        | H           |

\*\*a=water resistance; b=light fastness; c=weathering resistance; d=bending resistance; e=adhesion test; f=impact resistance; g=hardness.

of the painting materials used in the tests were as follows:

#### Composition 1

|                                        |                      |
|----------------------------------------|----------------------|
| Vehicle of the present invention       | 100 parts(by weight) |
| Epicoat 1001 (made by Shell Chemical)  | 66 "                 |
| Versamide 115 (made by Shell Chemical) | 34 "                 |
| Methyl isobutyl Ketone                 | 60 "                 |

#### Composition 2

|                                       |                      |
|---------------------------------------|----------------------|
| Vehicle of the present invention      | 100 parts(by weight) |
| Epicoat 828 (made by Shell Chemical)  | 200 parts(by weight) |
| Diethylene triamine                   | 26 "                 |
| 2,4,6-(tri-dimethylaminomethyl)phenol | 2 "                  |
| Diocetyl phthalate                    | 10 "                 |

The properties of the painted material after baking are shown in Table 1.

The properties of the painted material after baking are shown in Table 2, and as shown in the table, they were very excellent.

35 The above test was made according to JIS K-5400.

#### EXAMPLE 6

Each of vehicles A, B and C prepared in Examples 1, 2 and 3, respectively, was blended with a urethane resin (as shown below) to provide a urethane resin painting material. The composition of the painting material is as follows:

| Vehicle | Compo-<br>sition | Test method                       |                            |                                |                         |                            |                                                           |             |
|---------|------------------|-----------------------------------|----------------------------|--------------------------------|-------------------------|----------------------------|-----------------------------------------------------------|-------------|
|         |                  | **a                               | b                          | c                              | d                       | e                          | f                                                         | g           |
|         |                  | One year<br>in distilled<br>water | Fade-O-meter<br>2,000 hrs. | Outdoor exposure<br>for 1 year | 1/8" mandrel<br>100/100 | Du pont type, 1 kg.-50 cm. |                                                           | Pen-<br>cil |
| A.....  | 1                | Unvaried                          | No change in color         | No change in color             | Endured                 | Passed                     | Neither cracked nor stripped by the impact of the weight. | 2 H-H       |
| B.....  | 1                | do                                | do                         | do                             | do                      | do                         | do                                                        | 2 H-H       |
| C.....  | 1                | do                                | do                         | do                             | do                      | do                         | do                                                        | 2 H-H       |
| A.....  | 2                | do                                | do                         | do                             | do                      | do                         | do                                                        | H           |
| B.....  | 2                | do                                | do                         | do                             | do                      | do                         | do                                                        | H-HB        |
| C.....  | 2                | do                                | do                         | do                             | do                      | do                         | do                                                        | H-HB        |

45 The properties of the painted material after baking are shown in Table 1.

#### Composition 4

|                                            |                      |
|--------------------------------------------|----------------------|
| Vehicle of the present invention           | 100 parts(by weight) |
| Olester C-1,000 (Mitsui Toatsu-Kagaku Co.) | 50 "                 |
| Colonate L (Hodogaya Chemical Co.)         | 90 "                 |
| Ethyl acetate                              | 5 "                  |

The properties of the painted material after baking are shown in Table 1.

TABLE 1

| Vehicle | Compo-<br>sition | Test method                       |                            |                                |                         |                            |                                                           |             |
|---------|------------------|-----------------------------------|----------------------------|--------------------------------|-------------------------|----------------------------|-----------------------------------------------------------|-------------|
|         |                  | **a                               | b                          | c                              | d                       | e                          | f                                                         | g           |
|         |                  | One year<br>in distilled<br>water | Fade-O-meter<br>2,000 hrs. | Outdoor exposure<br>for 1 year | 1/8" mandrel<br>100/100 | Du pont type, 1 kg.-50 cm. |                                                           | Pen-<br>cil |
| A.....  | 1                | Unvaried                          | No change in color         | No change in color             | Endured                 | Passed                     | Neither cracked nor stripped by the impact of the weight. | 2 H-H       |
| B.....  | 1                | do                                | do                         | do                             | do                      | do                         | do                                                        | 2 H-H       |
| C.....  | 1                | do                                | do                         | do                             | do                      | do                         | do                                                        | 2 H-H       |
| A.....  | 2                | do                                | do                         | do                             | do                      | do                         | do                                                        | H           |
| B.....  | 2                | do                                | do                         | do                             | do                      | do                         | do                                                        | H-HB        |
| C.....  | 2                | do                                | do                         | do                             | do                      | do                         | do                                                        | H-HB        |

45 \*\*a=water resistance; b=light fastness; c=weathering resistance; d=bending resistance; e=adhesion test; f=impact resistance; g=hardness

The properties of the painted material were measured, the results of which are shown in Table 3. As is clear from the results, the prepared painted materials showed excellent properties.

determined by nuclear magnetic resonance absorption spectrum, and a transparency such that the percent transmittance of a 10 percent hexane solution thereof, measured by the absorption of visible light of

TABLE 3

| Vehicle | Compo-<br>sition | Test method                              |                                 |                                      |                   |              |                                                           | Pencil |
|---------|------------------|------------------------------------------|---------------------------------|--------------------------------------|-------------------|--------------|-----------------------------------------------------------|--------|
|         |                  | **a<br>One year<br>in distilled<br>water | b<br>Fade-O-meter<br>2,000 hrs. | c<br>Outdoor exposure<br>for 1 year. | d<br>1/8" mandrel | e<br>100/100 | f<br>Du Pont type, 1 kg.-50 cm.                           |        |
| A       | 4                | Unvaried.                                | Not inferior to control sample. | Not inferior to control sample.      | Endured.          | Passed.      | Neither cracked nor stripped by the impact of the weight. | 2H-H   |
| B       | 4                | do                                       | do                              | do                                   | do                | do           | do                                                        | 2H     |
| C       | 4                | do                                       | do                              | do                                   | do                | do           | do                                                        | H      |

\*\*a=water resistance; b=light fastness; c=weathering resistance; d=bending resistance; e=adhesion test; f=impact resistance; g=hardness.

NOTE.—The above test was made according to JIS K-5400.

What is claimed is:

1. A paint vehicle comprising a hydrocarbon compound having a specific gravity of from 0.92 to 1.0, a mean molecular weight of from 200 to 1,000 measured by a vapor pressure osmotic pressure method, an aromatic C—H proton density of less than 3 percent, said aromatic C—H proton having a value of less than 4

wavelengths longer than 500 m $\mu$ , is higher than 60 percent wherein the softening point of said vehicle varies from 25° to 100° C as a solid and wherein the viscosity of said vehicle as a liquid at 25° C varies from 1,000 to 50,000 cps.

2. The paint vehicle of claim 1, wherein said percent transmittance is higher than 80 percent.